

May 2, 1961

W. B. WHITNEY

2,982,728

LUBRICATING ADDITIVE

Filed March 26, 1954



INVENTOR.  
W. B. WHITNEY

BY  
*Hudson & Young*

ATTORNEYS

1

2,982,728

## LUBRICATING ADDITIVE

William B. Whitney, Bartlesville, Okla., assignor to Phillips Petroleum Company, a corporation of Delaware

Filed Mar. 26, 1954, Ser. No. 418,803

10 Claims. (Cl. 252—39)

This invention relates to lubricating additives having 15 detergent and/or dispersant properties. In one of its more specific aspects, this invention relates to petroleum lubricating oil compositions. In another of its more specific aspects, this invention relates to methods of producing these lubricant additives.

As the speed and output of internal combustion engines have increased to higher and higher values, the ability of oils without additives to maintain an engine free from lacquer, sludge and carbon deposits has decreased. Under present day conditions, lubricating oils for use in automotive and diesel engines require the use of additive agents. Stop and go driving in cold weather also has a tendency to produce sludge in the lubricating system and additives are necessary to combat this problem.

The requirements desirable in a satisfactory detergent additive are: (1) compatibility with lubricating oil and other types of additives which may be present; (2) maintenance of satisfactory cleanliness of engine parts, principally in the ring belt zone of the piston; and (3) chemical inertness with respect to supplemental additives and metal engine parts. Additional desirable characteristics include: (1) ease of handling, either as such or as an oil concentrate; (2) minimum effect on oil properties, such as viscosity, color and odor; (3) inexpensive overall cost; and (4) independence with respect to critically limited or expensive raw materials.

The use of additives in lubricating compositions as corrosion inhibitors, oxidation inhibitors, viscosity index improvers, dispersing agents, pour-point depressants, extreme pressure agents, lubricity improvers and ash forming detergents, is well known. The need for additives to improve various specific properties of lubricating oils is all the more acute and necessary, in view of the service conditions which lubricating oils undergo and must withstand. In internal combustion engines, it is desirable that the lubricating compositions be resistant to sludge and varnish formation and in the event of such formation to prevent the deposition of these materials on the metallic parts of the engines.

Each of the objects of this invention will be obtained by at least one of the aspects of this invention.

An object of this invention is to provide improved lubricant additives having detergent and/or dispersant properties.

Another object of this invention is to provide new lubricating compositions containing the additives of this invention.

Another object of this invention is to provide a method for the production of additives suitable for use in lubricating oil compositions.

Another object of this invention is to provide a method for the preparation of petroleum lubricating oil compositions possessing excellent detergent properties.

Other and further objects of this invention will be apparent to those skilled in the art upon studying the accompanying disclosure.

2

Accompanying and forming a part of this specification is a drawing which illustrates apparatus which can be used in the practice of this invention.

I have now discovered that an additive for lubricating 5 oils which is useful as a detergent or dispersant therein can be produced by subjecting a selected hydrocarbon fraction having at least 40 carbon atoms per molecule to oxidation in the presence of alkaline earth compounds or by oxidizing such a hydrocarbon fraction and there- 10 after treating the oxidized material with alkaline earth metal compounds.

The additives prepared according to this invention are 15 readily incorporated in lubricating oils to form compositions of improved performance characteristics. Lubricants containing these additives exhibit excellent resistance to deposition of sludge and varnish in internal combustion engines operating both under high performance conditions and under intermittent service. They materially reduce ring-sticking, piston varnish, etc., in such engines 20 and impart cleanliness to the engine.

One material well suited for the production of my 25 detergent is preferably one which is substantially saturated containing at least 40 carbon atoms per molecule, preferably between 40 and 80 carbon atoms per molecule. 30 The hydrocarbon material should have a refractive index of between 1.440 and 1.520. Hydrocarbon materials which can be satisfactorily used in the preparation of my detergent include substantially saturated diene polymers, such as polybutadiene and polypentadiene, and 35 polymers of olefins having from 2 to 12 carbon atoms per molecule, such as polypropylene, polyethylene, polyisobutylene, etc., preferably having a ratio of carbon atoms to olefin bonds of at least 40 to 1 and not less than 16 to 1, copolymers such as styrene-olefin copolymers, alkylated polystyrene, and a petroleum lubricating oil fraction, which has substantially no asphalt, either in its natural state or when deasphalted, and which has been solvent extracted to reduced the content of aromatic-type hydrocarbons therein and preferably dewaxed.

The detergent-type lubricating oil additives of this 40 invention can be used alone or in combination with other additives. Infrared spectrograms of these materials reveal the presence of groups characteristic of substantially neutral completely organic, oxygen-containing compounds 45 such as alcohols, ethers, esters, lactones, anhydrides, ketones, and aldehydes. Examination of the oxidized materials by infrared spectroscopy discloses very marked changes in the absorption bands upon oxidation of the 50 selected hydrocarbon fractions disclosed herein. A strong carbonyl band within the 5.75 to 5.87 micron region is produced in the initial oxidation of the hydrocarbon as is a weak absorption band at 2.94 to about 3.0 microns which indicates the presence of a low concentration of 55 hydroxyl groups. These bands are characteristic of a concentrated oxidized product but also appear in the scanning of the total oxidized hydrocarbon fraction. The concentrated oxidized material also exhibits a broad absorption band in the 7 to 10 micron region, this band being much weaker for the unconcentrated material.

Petroleum fractions which are suitable for production 60 of the material of this invention, i.e., an excellent detergent for use in lubricating oils, include Pennsylvania, Mid-Continent, California, East Texas, Gulf Coast, Venezuela, Borneo, and Arabian crudes. The source of the crude from which the petroleum fraction is derived does not significantly influence the preparation or properties 65 of the detergent material of this invention, provided the petroleum fraction has been prepared by subjecting the crude to certain necessary treatments to exclude undesired materials therefrom.

In the preparation of the preferred petroleum frac-

tion from which the detergent material of this invention is produced, a crude oil is topped, i.e., distilled to remove therefrom the more volatile, lower molecular weight hydrocarbons, such as gasoline and light gas oil, and then vacuum reduced to remove heavy gas oil and light lubricating oil of the SAE 10 and 20 viscosity grade. The vacuum reduced crude is then propane fractionated to remove an overhead fraction of about 100 SUS at 210° F. viscosity and the residual material is subjected to a second propane fractionation to remove another overhead fraction of about 200 SUS at 210° F. viscosity. The residue from the second fractionation may be subjected to a third propane fractionation to remove still another overhead fraction of about 575 SUS at 210° F. viscosity. Propane fractionation may be modified by the presence of butane, ethane or methane to the extent desired.

Following the propane fractionation step, the overhead oil fraction is solvent extracted with a selective solvent which will separate the paraffinic hydrocarbons from the more aromatic-type hydrocarbons. Suitable selective solvents for aromatic hydrocarbons include among others, the various phenols, sulfur dioxide, furfural and  $\beta,\beta$ -dichlorodioethyl ether. This solvent extraction step for the removal of the more highly aromatic compounds can be carried out in accordance with the well-known concurrent or countercurrent solvent extraction techniques, as well as by the Duo-Sol technique.

The resulting solvent extracted material, before or after the removal of the more aromatic hydrocarbons, is preferably dewaxed. Dewaxing may be carried out by any conventional method, e.g., by solvent dewaxing using propane or solvent mixtures, such as methyl ethyl ketone or methyl isobutyl ketone with benzene at a suitable temperature.

Each fraction of the phenol extracted, dewaxed, propane-fractionated oil can be used in preparing the detergent material of this invention with good results but the oil fraction from the second propane fractionation is preferred. It will be recognized by those skilled in the art that propane fractionated oils differing from those described may be used or a single broad viscosity cut can be used. The residual material from the final propane fractionation contains the rejected asphalt and more aromatic oils.

Although the preferred method for preparation of feed stock is as above described, other methods may be used to secure a similar type hydrocarbon fraction. Thus, a vacuum reduced crude which has essentially no asphalt, such as a Pennsylvania oil, may be used directly or after a light acid treatment. Another method, while not feasible commercially at the present time, is ultra-high vacuum (molecular) distillation to obtain the desired fraction.

As pointed out above, a polydiene, such as liquid polybutadiene which is prepared by sodium-catalyzed polymerization of butadiene and which material is subsequently hydrogenated so as to reduce the olefinic unsaturation thereof to the desired amount, is another suitable feed stock for use in the production of the detergent material of this invention. When butadiene is polymerized, only one double bond remains therein for each butadiene group of the polymer. The feed material of this invention should be hydrogenated sufficiently so that the ratio of carbon atoms to double bonds is at least 16 to 1. Preparation of liquid polybutadiene may be carried out by means of the process set forth in U.S. Patent No. 2,631,175, issued March 10, 1953, by W. W. Crouch.

Another suitable feed stock is a liquid or semi-solid polybutadiene which is prepared by conventional emulsion polymerization and coagulation to form synthetic rubber, subsequently hydrogenating said material so as to reduce the olefinic unsaturation thereof to the desired amount and finally thermally depolymerizing it suffi-

ciently to increase the ease of oxidation and to increase the oil solubility.

Another suitable feed material is a high molecular weight polymer prepared by zirconium tetrachloride polymerization of propylene. Still another material which has proved to be useful as a feed material for the oxidation step in the preparation of the detergent material of this invention is a "tacky polymer" prepared by the polymerization of propylene over chromia-silica-alumina catalyst, as more fully disclosed in U.S. application Serial No. 333,576, filed January 23, 1953, now abandoned, by John P. Hogan and Robert L. Banks. Another suitable feed material is a copolymer of styrene with olefins in which the olefin portion constitutes at least 50 percent of the total molecular weight of the molecule. With any of these feed materials, it is desired to reduce the amount of olefinic unsaturation to such an extent that the ratio of carbon atoms to olefinic bonds is preferably at least 40:1 and not less than 16:1. The hydrocarbon stocks which are useful in the practice of this invention include those materials which are identifiable as having the following properties set forth in Table I.

TABLE I

|    | Property                                         | Broad range | Preferred Range |
|----|--------------------------------------------------|-------------|-----------------|
| 30 | Refractive Index $n_{D}^{20}$                    | 1.440-1.520 | 1.480-1.515     |
|    | Average Molecular Weight                         | above 550   | 600-10,000      |
|    | Minimum Molecular Weight                         | 450         |                 |
|    | Viscosity, SUS at 210° F                         | above 50    | above 100       |
|    | Viscosity Index (when determinable) <sup>1</sup> | 50-125      | 80-120          |
|    | Carbon Atom Content per Molecule                 | above 40    | 50-720          |

<sup>1</sup> Viscosity index not determinable for non-Newtonian materials.

Lubricating oils which are suitable as feed stock in my process have the properties set forth in Table II.

TABLE II

|    | Property                         | Broad range | Preferred Range |
|----|----------------------------------|-------------|-----------------|
| 40 | Refractive Index $n_{D}^{20}$    | 1.440-1.520 | 1.480-1.515     |
|    | Average Molecular Weight         | 550-1300    | 600-900         |
|    | Minimum Molecular Weight         | 450         |                 |
| 45 | Viscosity, SUS at 210° F         | 50-1400     | 100-600         |
|    | Viscosity Index                  | 50-125      | 80-120          |
|    | Carbon Atom Content per Molecule | 40-80       | 50-70           |

During oxidation, scission takes place in the large hydrocarbon molecules, the lighter products being collected in traps. When nitrogen gas was passed through the untreated oil at 250° C. substantially no volatile products were collected. Only a very small amount was collected when the temperature was raised to 300° C., thus demonstrating that the major cause of the formation of the volatile products is oxidation and not thermal decomposition nor stripping of light ends originally present in the oil. With oils of moderate molecular weight, scission cannot take place in any position but what one or all of the fragments is sufficiently small that distillation takes place, thus preventing accumulation of molecules appreciably smaller than those originally present. Hence the viscosity is not decreased to any great extent. Concomitant with the oxidative scission reaction, there is a polymerization or condensation reaction resulting in an increase in viscosity. The net change in viscosity is apparently due to the relative magnitude of each reaction. In very high molecular weight hydrocarbons, the oxidative scission more frequently results in fragments too large to be removed by distillation and, hence, the average molecular weight decreases, tending to cause a decrease in viscosity. As the oxidation reaction proceeds, the reactions causing increased molecular weight may overcome, more or less, those causing a decrease in molecular weight. As a result, the molecular

Weights of charge oils having molecular weights in the lower range tend to increase and those in the higher range tend to decrease during the initial oxidation period.

If desired, the petroleum oil fraction which has been highly refined, as described above, may be further subjected to additional refining treatments. For example, these petroleum fractions may be hydrogenated to convert any aromatic compounds therein to the corresponding naphthenic and saturated hydrocarbon, or if desired, these petroleum fractions may be subjected to contact with adsorbents such as silica gel for the preferential adsorption and removal of the more aromatic hydrocarbons therefrom. Generally, the petroleum fraction which is oxidized for the production of the detergent of this invention should contain not more than 20 percent of the carbon atoms in aromatic rings, as determined by the ring analysis described in the book *Aspects of the Constitution of Mineral Oils* by K. Van Nes and H. A. Van Westen, Elsevier Press, New York City, New York. It is preferred that the aromatic content of the petroleum fraction be reduced to an economically feasible extent by refining procedures since oxidation of aromatic-type hydrocarbons tends to result in the formation of oil-insoluble products not suitable for the present invention. It also appears that aromatic constituents oxidize more readily than do the non-aromatic components. Thus, failure to remove materials containing a high percentage of carbon atoms in aromatic rings from the feed before oxidation results in formation of considerable oil-insoluble materials. Usually, a suitable petroleum fraction, upon distillation under reduced pressure, e.g., molecular distillation, will produce a first 10 percent by weight fraction which has a viscosity of more than 50 SUS at 210° F., preferably more than 80 SUS at 210° F.

In one method of carrying out my invention, the hydrocarbon fraction is oxidized and then treated with the alkaline earth compound. During the oxidation reaction, the hydrocarbon fraction is modified, resulting in a product of increased dispersing activity which differs from the starting material in respect to the following four physical characteristics: (1) an increase in the carbon to hydrogen weight ratio; (2) usually an increase in molecular weight; (3) an increase in the oxygen content; and (4) a decreased solubility in propane under propane fractionating conditions.

All these changes are brought about by contacting an above-described selected hydrocarbon fraction under suitable conditions of temperature and pressure with an oxidizing agent, such as free oxygen, sulfur trioxide, nitrogen dioxide, nitrogen trioxide, nitrogen pentoxide, acidified chromium oxides and chromates, permanganates, peroxides, such as hydrogen peroxide, sodium peroxide and ozone. Any oxygen-containing material capable of releasing free oxygen under the oxidizing conditions can be used. Nitric acid can be used. Other suitable oxidizing agents include air, relatively pure commercial grade oxygen, oxygen enriched air, and a mixture of oxygen with an inert gas, such as carbon dioxide and nitrogen. Even oxygen admixed with natural gas or methane is satisfactory. Air having less than the usual amount of oxygen may also be used. Air is economically a preferred oxidizing agent.

Generally, the oxidation reaction is carried out at a temperature in the range of from -40° F. to 800° F. When using an active oxidizing agent, such as sulfur trioxide, temperatures in the range of -40° F. to 400° F., preferably 70° F. to 200° F., are used. With less active oxidizing agents, such as air, higher temperatures are used, such as 100° F. to 800° F., preferably 375° F. to 575° F. Higher oxidation temperatures result in a faster oxidation reaction. When the oxidizing agent is in the gaseous phase, another variable which affects the rate of the oxidation reaction is the partial pressure of the oxidizing agent. Accordingly, as the pressure at which the oxidation reaction is carried out is increased, other con-

ditions remaining the same, the oxidation reaction proceeds at a faster rate. Therefore, depending upon the rate of oxidation desired, the oxidation reaction is carried out at sub-atmospheric, atmospheric or super-atmospheric pressures. Usually it is preferred to carry out the oxidation reaction at a pressure between about 10 and 100 pounds per square inch absolute, depending upon the composition or oxygen content of the oxidizing gas. Lower or higher absolute pressures may be satisfactorily used, if desired. Lower oxidation pressures are useful, in that they facilitate release and removal of the more volatile, and other undesirable materials, e.g., H<sub>2</sub>O, from the reaction mixture.

The rate of oxidation is also dependent upon, and influenced by, the distribution of the oxidizing gas within the reaction mixture and the rate of introduction of the oxidizing gas thereto. The oxidizing agent is preferably introduced and present in the reaction mixture in a finely dispersed state, in order to achieve better contact with the materials undergoing oxidation and better mixing therewith. An increase in the rate of introduction of the oxidizing gas, of course, increases the rate of oxidation, other conditions remaining unchanged. The conditions of temperature, pressure, oxygen content of the oxidizing gas, rate of introduction of oxidizing gas, etc., are correlated, adjusted and controlled so as to carry out the oxidation reaction at a sufficiently rapid rate so as to minimize reaction time while readily and easily controlling the reaction.

Conditions which have been found to be satisfactory for producing the detergent of this invention from a selected hydrocarbon fraction, when using a moderate oxidizing agent, such as air, are set forth in Table III.

TABLE III

|    | Reaction Condition                                                                                     | Broad Range | Preferred Range |
|----|--------------------------------------------------------------------------------------------------------|-------------|-----------------|
| 40 | Temperature.....°F                                                                                     | 100-800     | 375-575         |
|    | Time of Oxidation.....hrs.                                                                             | 3-75        | 5-50            |
|    | Pressure.....p.s.i.a.                                                                                  | 10-200      | 15-100          |
|    | Rate of introduction of oxidizing agent in s.c.f. (standard cubic feet) per pound of oil per hour..... | 0.01-3.0    | 0.04-0.4        |

Exemplary of the influence of various variables upon the oxidation reaction, it is pointed out that at a temperature of 482° F. and at an air introduction rate of about 0.32 s.c.f. per pound of oil per hour and at about atmospheric pressure, the oxidation reaction requires about 20 hours before the desired degree of completion is reached (as measured by increase in viscosity). When the air rate was increased to 1.44 s.c.f. per pound of oil per hour, only 16 hours were required to convert the oil to an oxidized product of similar viscosity. Increasing the reaction temperature to 572° F. decreased the time required for oxidation appreciably. Reducing the reaction temperature to below 390° F. increased the reaction time under these conditions.

It has been found that the time required for the reaction mixture to reach the desired degree of oxidation can be decreased or increased by the use of catalysts. Positive (promoters) or negative (inhibitors) catalysts can be used to modify the reaction rate and time.

Catalysts which have been found to promote the oxidation reaction and to decrease the time required for oxidation reaction include the various well known oxidation catalysts, such as the oil soluble salts and compounds containing such metals as copper, iron, cobalt, lead, zinc, cadmium, silver, manganese, chromium, vanadium, and the like, having an atomic number between 51 and 113, inclusive. The naphthenates of these metals are particularly useful. Especially useful and outstanding as a catalyst are those compounds which are obtained by reacting a compound containing both phosphorus and sulfur, such as P<sub>2</sub>S<sub>5</sub>, with a terpene, either

monocyclic or dicyclic or a mixture thereof, such as pinene, as disclosed in my copending U.S. application, Serial No. 264,839, filed January 3, 1952, now U.S. Patent No. 2,758,069. A particularly effective catalyst of this type is widely used as a corrosion inhibitor for petroleum lubricating oils and is sold under the trade name Santolube 395-X, and is a  $P_2S_5$ -terpene reaction product. This reaction product exhibits a marked catalytic effect, resulting in a decrease of several hours in the time normally required for the oxidation reaction to reach the desired degree of completion. Also, it is pointed out that the above-mentioned metal naphthenates, especially the copper and iron naphthenates, effectively catalyze the oxidation reaction at a temperature in the range of 300° to 500° F. Usually, however, the catalytic effect of these metal naphthenates is pronounced for only a few hours and then becomes ineffective, the addition of more naphthenates being required in order to maintain a catalytic effect upon the oxidation reaction.

Negative catalysts or inhibitors, i.e., materials which tend to increase the time required for the oxidation reaction, are usually high molecular weight aliphatic alcohols, such as the  $C_{16}$  to  $C_{24}$  highly branched, non-straight chain and normal aliphatic alcohols. Typical material useful as an anti-catalyst or inhibitor is a highly branched octadecyl alcohol, such as 2,2,4,5,8,10,10-heptamethyl-5-undecanol and n-octadecyl alcohol.

These catalysts can be added in catalytic amounts, usually in the range of 0.1 percent to 4.0 percent by weight of the oil undergoing oxidation, depending upon the catalytic promoting or inhibiting effect desired. An amount of one of these types of catalyst, such as about 1.0 percent by weight of the oil, is sufficient for most purposes. It is pointed out that the employment of catalysts is beneficial, in that they decrease or increase the time required for oxidation (for better control) and, in some cases, even improve the quality of the detergent recovered as a product from the oxidation reaction. However, the presence of a catalyst, positive or negative, is not essential to the practice of this invention.

More active oxidizing agents, such as sulfur trioxide, may also be used in the oxidation step, as pointed out above. When liquid sulfur trioxide is utilized as the oxidizing agent, the reaction is most readily carried out when both the oil and sulfur trioxide are separately diluted with a modifying solvent. Solvents which may be utilized in this operation under suitable temperature conditions include liquid sulfur dioxide, hexane, tetrachloroethylene, ethylene dichloride, pyridine, nitrobenzene and dioxane.

Liquid sulfur trioxide is an extremely reactive compound and, if added directly to the oil, will cause excessive charring and violent splattering. It is necessary to moderate this excessive reactivity by dilution with a solvent, such as those disclosed above. A molar ratio of solvent to sulfur trioxide of at least about 1:1 appears to be necessary, and it is preferred to use a ratio of 2:1 or greater. Dilution of the oil is also very desirable for the reduction of viscosity and to facilitate mixing, but such dilution is not required. Dilution of the oil may be obtained with some non-reactive solvent other than that utilized for the dilution of the sulfur trioxide. Use of the same diluent, however, simplifies the recovery problem. Gaseous  $SO_3$  may be introduced into the oil directly or mixed with a carrier gas, such as air, nitrogen or other inert gas. In the case of gaseous  $SO_3$ , an elevated temperature, e.g., 200 to 300° C., is frequently used.

The extent of oxidation is determined by the ratio of oil to sulfur trioxide. The weight ratio may be varied from 1:1 to 30:1, but is preferably maintained within the range of between 3:1 to 18:1. Ratios from 3:1 to 8:1 are the most desirable. Very low ratios result in the use of excessive amounts of sulfur trioxide without obtaining a corresponding increase in useful product. Very

high ratios fail to obtain sufficient oxidation to be economical.

The initial reaction of the sulfur trioxide with oil is almost instantaneous at room temperature or above, but 5 the reaction continues for extended periods of time, e.g., up to as much as 144 hours or more. At higher temperatures the time of the slower secondary reactions is shortened to less than 24 hours. The evolution of sulfur dioxide and other gases causes much foaming and 10 the rate of reaction must be controlled sufficiently to permit the capacity of the apparatus to handle the foaming reaction mixture. The time required for reaction may be shortened to as little as three minutes, in which case, secondary reactions do not take place to any great extent. The quality of the product is not materially affected by the length of reaction time or by the absence or occurrence of the secondary reactions.

The temperatures which may generally be utilized in the oxidation reaction, wherein sulfur trioxide is used as 20 the oxidizing agent, range from -40° to 400° F., preferably from 70° F. to 200° F. A very short period of time, usually less than three hours, is required for the initial reaction. This time is sometimes as short as three minutes.

25 After the reaction, the product is treated for the removal of acid and other impurities. Acid is conveniently removed from the product by water washing. The product is concentrated in the manner discussed later in connection with the product obtained in a process utilizing a less active oxidizing agent.

The detergent produced by sulfur trioxide oxidation is somewhat improved in color by reduction. This is preferably accomplished by treatment in alcohol with lithium hydride or with zinc and hydrochloric acid. Catalytic hydrogenation or chemical reduction can also be used.

30 The extent to which the oxidation reaction is carried out is dependent upon the selected oil fraction being oxidized and the yield of detergent material desired. I 40 have found that if the oil being oxidized contains a relatively low concentration of lower molecular weight hydrocarbons, the oil may be oxidized to a considerable extent, up to as high as 75 percent by weight of the oil charged, without any deleterious effects upon the reaction itself or the detergent product. Also, I have observed 45 that when the aromatic content of the charge stock is low, such as below about 5 percent by weight of carbon atoms in aromatic rings and especially below about 2 percent by weight, the charge stock can be oxidized to 50 a greater extent without any undesirable effects or adversely affecting the yield, such as may happen when there is an appreciable amount, above about 5 percent by weight of aromatic carbon atoms, present therein. In general, the oxidation reaction is carried out until the 55 oxidized oil has increased in viscosity, when expressed in Saybolt Universal Seconds (SUS) at 210° F., from 1.5 to 50 fold, preferably from 1.5 to 10 fold, over that of the originally charged unoxidized oil. The range 1.5 to 2 fold has been found especially valuable with some stocks.

60 When the oxidation reaction is carried out to a 3 to 10 fold increase in viscosity, the yield of active detergent recovered from the oxidized oil amounts to about 15 to 50 percent by weight of the original unoxidized oil. Continued oxidation, especially to yields above about 60 percent, tends to produce a certain amount of oil-insoluble 65 oxidized materials which, although they do not adversely affect the effectiveness of the oil-soluble detergent, do adversely affect the yield of the desired product. Also, since it is often necessary to remove these oil-insoluble 70 oxidized materials, it is desirable, therefore, not to continue the oxidation reaction beyond that point at which the oil-insoluble materials are produced.

In general, however, the extent to which the selected oil fraction is oxidized in the practice of this invention 75 is primarily a matter of convenience, based on the ease

of handling of reactants and reacted (oxidized) materials, yield desired, and recovery and purification steps contemplated in the production of the desired product. Illustrative of this, it has been found that after carrying out the oxidation reaction and the oil and product are separately recovered from the reaction mixture, the recovered oil can be again oxidized to produce an additional product which is at least equal to and often superior in quality and effectiveness as a lubricating oil detergent additive over the first produced product. Also, it has been found that after completion of the oxidation reaction and the product recovered (as by propane fractionation of the oxidation reaction mixture), if the recovered product is again oxidized to a hard, brittle mass, the reoxidized material has a detergent power or activity, when tested as a lubricating oil additive, by a hereinafter defined test, in a Lauson engine which simulates the well-known, widely accepted L-1 diesel engine test, only slightly less than the product recovered from the initial and first oxidation reaction.

While the viscosity increase measured at SUS at 210° F. has been stated as one way of determining and measuring the extent of the oxidation reaction, it is not the only way. Another way is to measure the amount of water produced during the oxidation reaction. Another method of determining the extent of the reaction is to measure the detergent activity of the oxidation reaction mixture by a spot plate test. Still another method is to determine the amount of propane insoluble material present in the oxidation reaction mixture. When the oxidation reaction is completed to the extent desired, the propane insoluble, oil soluble material in the reaction mixture amounts to between about 5 and about 60 percent by weight of the reaction mixture, more often between about 15 and about 40 percent by weight.

The oxidation reaction mixture, after oxidation, can be used directly without additional concentration or purification. However, if a product of improved quality, purity and greater concentration and effectiveness per unit weight is desired, the active detergent oil-additive material is preferably removed and recovered from the oxidation reaction mixture. When the hydrocarbon feed to the oxidation reaction is a liquid, the recovery and concentration of the active additive material is preferably obtained by propane fractionation, such as is disclosed by J. M. Whitely and G. A. Beiswenger in U.S. Patent 2,110,845.

Following propane fractionation the material is a firm, plastic or slightly brittle mass soluble in pentane, benzene, diethyl ether and the other usual liquid hydrocarbon solvents. It is also soluble in all petroleum lubricating oils, as well as in polymers and polyester synthetic oils. The additive leaves a dark red color, when rubbed on a white surface and when dissolved in a lubricating oil, such as a motor oil, gives the oil a black appearance by reflected light. The oxidized material has a strong tinting power when dissolved in lubricating oil. It has a low acid number below about 50, expressed as the number of milligrams of KOH per gram, and a saponification number between 0 and about 100. The oxygen content of these materials ranges from about 2 percent up to about 10 percent by weight, usually from 3 percent to 8 percent, although in some cases the oxygen content may be as high as 15 percent or as low as 1 percent by weight.

While these solid oxygen-containing materials appear to have a superficial resemblance to resins, asphaltenes and sludges heretofore reported in the literature, there are a number of distinct and fundamental differences thereto. These materials, such as sludges, asphaltenes and resins, are characterized by insolubility in light hydrocarbons, have a high acid number, in some cases as high as 180, and also possess high saponification values, usually above 300 and even as high as 450. In contrast thereto, these materials are soluble in light hydrocarbons,

have an acid number below about 50 and a saponification number below about 100.

Following the oxidation, an alkaline earth material, such as the oxides, hydroxides and carbonates of calcium, strontium or barium, is added. Representative compounds include calcium oxide, calcium hydroxide, calcium carbonate, barium oxide, barium hydroxide, strontium hydroxide, and strontium carbonate. This is preferably done by dissolving the oxidized material in a suitable solvent, such as an SAE 10 oil, and adding the alkaline earth compound. Other solvents include aromatics, such as benzene and toluene. Frequently it is advantageous to add a small amount of a non-solvent, such as isopropyl alcohol, in order to obtain better contacting. This is especially true when an aqueous solution of the alkaline earth material is used. When the alkaline earth hydroxide is used, the hydrate may likewise be used, i.e., when barium hydroxide is used, the anhydrous material, the monohydrate, or the octahydrate, can be used. The alkaline material is added as an aqueous solution or as finely powdered material, in a concentration of 0.1 to 20 weight percent, and preferably from 0.5 to 10 weight percent of the hydrocarbon material. Following addition, the mixture is preferably stirred for a sufficient length of time to insure adequate reaction. The resulting solution is filtered to remove excess alkaline metal material and any other insoluble material. Temperatures for this reaction usually range from around 50° F. to around 500° F., although the preferred temperature range is 200 to 300° F. A reaction time of 5 minutes to 5 hours is usually required. The resulting product, after filtration, is an oil concentrate containing the additive, which can be added to any desired lubricating oil base stock direct, or the additive may be separated from the oil concentrate.

Another method of preparing these additives is to add the alkaline earth compound to the hydrocarbon fraction prior to the oxidation step. In this manner, the additive can be prepared in one step. The physical conditions of temperature and pressure set forth above for the oxidation are used for the reaction in this case.

This active solid detergent material can be recovered directly from the reaction mixture by solvent extraction with a solvent which is selective for the relatively unoxidized, essentially hydrocarbon material therein, and which solvent is at the same time essentially a non-solvent for the active detergent material in the reaction mixture. Suitable solvents for the recovery of the solid active detergent material from the oxidized reaction mixture include propane, isopropyl alcohol, a solvent mixture of propane with modifying amounts (up to about 50 percent by weight) of other low boiling hydrocarbons, such as methane, ethane, and butane. Other selective solvents, such as methyl ethyl ketone, methyl isobutyl ketone, tertiary butyl alcohol, isobutyl alcohol, ethyl acetate, dioxane, morpholine, dimethyl formamide and phenol, are also useful. In general, those polar compounds containing only carbon, hydrogen, and oxygen atoms, such as aliphatic alcohols, aliphatic ketones, and esters having from 3 to 8 carbon atoms per molecule, are useful as treating materials in the practice of this invention. Mixtures of these various materials may be used.

One step-wise process for concentrating the detergent material comprises extracting the partially oxidized oil with methyl isobutyl ketone, methyl ethyl ketone, or mixtures of the two, at appropriate temperatures so as to dissolve only the oil and lower molecular weight additive material. The proper temperature will depend upon the ratio of solvents and the percentage of product to be dissolved. The undissolved material is thereafter mechanically separated from the dissolved material.

When these materials are used in obtaining the active detergent material from the oxidized reaction mixture, the active solid detergent is recovered as a propane insoluble, oil soluble, solid phase (raffinate), the ineffective,

substantially hydrocarbon material of the reaction mixture being dissolved in the treating material as an extract. The propane soluble phase, from which the active detergent material is separated, has a viscosity index much higher than that of the unoxidized oil. This propane soluble phase may be used to blend with an oil for the purpose of improving the viscosity index of that oil.

In the recovery of the active detergent material, it is preferred in the practice of this invention to employ propane as a selective solvent, the solid active detergent being recovered as a separate propane insoluble phase under propane fractionating conditions of temperature, pressure and ratio of solvent to material being treated (usually 5:1 to 25:1 by volume). The solvent extraction operation for the recovery of the active detergent material is usually carried on at a temperature in the range 50° F. to 250° F., especially in the range 100° F. to 160° F., and a pressure of between 200 p.s.i.g. to 500 p.s.i.g. Countercurrent solvent extraction techniques are usefully employed, as well as multiple, solvent extraction steps of separately contacting and recovery of the undissolved active detergent.

In many instances, the activity of the detergent material is considerably increased by additionally treating this recovered solid detergent material with an aliphatic alcohol, in the C<sub>3</sub> to C<sub>8</sub> range, such as isopropyl alcohol, and recovering a purified and more active detergent therefrom as a solid, alcohol insoluble phase. The alcohol treatment has a two-fold purpose. Traces of peroxides, aldehydes, and the like, which may be oxidation products, are removed thereby. In addition thereto, it appears that a beneficial chemical change takes place during stripping of residual alcohol solvent from the additive material.

The above-described sequence of recovery and purification steps does not in some instances greatly influence the quality and effectiveness of the solid, final detergent product. It is preferred to employ a propane fractionation step prior to the organic polar compound treating step to avoid emulsions which are difficult to break and which present operational difficulties when the alcohol or ketone treating step precedes the propane solvent extraction step.

The method by which the additives of the present invention are formed is not fully understood, since the amount of alkaline earth metal compound reacting often exceeds by a large factor that corresponding to the neutralization number. The reaction appears to be quite rapid, indicating the saponification of ester groups is not the full explanation. While not wishing to be bound by any possible theory set forth, I believe that it may be that chelates or other coordination complexes play an important part.

The material prepared from the oxidation of the oil in the presence of an alkaline earth metal compound, such as barium hydroxide, has excellent detergent properties, as measured by the spot plate test, even when very little viscosity increase has taken place. Measurement of the off-gas indicates that oxidation is taking place during the reaction even though the viscosity of the oil is not increasing rapidly.

The oxidation step disclosed herein is similar to that disclosed in my copending application Serial No. 304,659, filed October 15, 1952, now abandoned, and reference is made thereto for further details and illustrative examples. The additives of this invention show improvements over the additives produced according to the method of Serial No. 304,659 in certain respects when tested in a paraffinic oil in an engine using a dirty fuel.

The oil to which the solid active detergent material of this invention is added can be any oil of lubricating viscosity and, preferably, is a lubricating oil commonly used in internal combustion engines, such as in the crankcase thereof. The additive is usually added to the base lubricating oil in effective detergent amounts and gen-

erally comprises between 0.1 percent to 10 percent by weight of the total lubricating oil composition, but may be as high as 25 percent for extreme service conditions. Usually, however, an amount in the range 0.3 percent to 10.0 percent by weight of the total lubricating oil composition is sufficient.

The modified diesel L-1 test referred to in the following examples was carried out for a shorter period of time than the 480 hours prescribed by the full scale diesel L-1 test set forth in "C.R.C. Handbook 1946" by the Coordinating Research Council, Inc., at pages 347 and following. The procedure outlined in the C.R.C. Handbook was modified as to the specific fuel. In its distillation characteristics, the fuel utilized in the tests set forth in the following examples had a 90 percent distillation of 600° F. to 640° F., a minimum 50 percent distillation of 500° F., and an endpoint of 650° F. to 690° F. The sulfur content in the fuel utilized had a minimum of .35 percent natural sulfur and a cetane number of between 40 and 45.

The simulated L-1 Lauson engine test, used in connection with the following examples, is described in "Motor Oils and Engine Lubrication" by Carl W. Georgi at page 83 and following. The operating conditions which were utilized in the tests of the following examples have been modified and are as follows.

The lubricating oil employed as a base oil in these tests was a solvent-refined Mid-Continent oil of lubricating viscosity and having the following characteristics

|    |                       |      |
|----|-----------------------|------|
| 30 | Gravity, API          | 30.3 |
|    | Viscosity at 210° F.  | 61.8 |
|    | Viscosity index       | 98   |
|    | Neutralization number | 0.01 |

The detergent in selected amounts was added to the base oil and tested in a standard Lauson engine. The test consisted in placing 920 grams of the base oil containing this detergent in the crankcase of a single cylinder Lauson gasoline engine. The engine was operated under a 1.2 horsepower load at 1600±20 r.p.m., maintaining a cooling jacket temperature of 300° F., an oil temperature of 225° F., an air-to-fuel ratio of 13.5:1, carburetor air at room temperature, spark advance of 25° before top of dead center, and crankcase vacuum of 1.0 inch of mercury. At the end of 60 hours' engine operation under these conditions, the engine was stopped, disassembled, and the piston, crankcase and bearings were examined. The piston varnish was rated on an arbitrary scale of 0 to 10 with 10 representing a clean or perfect condition and 0 representing the dirtiest condition.

#### Example I

##### PREPARATION OF ADDITIVE Ba(OH)<sub>2</sub> PRESENT DURING OXIDATION

A Mid-Continent oil, solvent refined, and dewaxed, having a viscosity of 208 SUS at 210° F. was oxidized by passing air into 3440 grams of the oil containing barium hydroxide octahydrate, equivalent to 2.0 percent barium hydroxide. The air was dried, metered and introduced through a porous plate located near the bottom of the oil. The oil containing the barium hydroxide was heated to 482° F. and treated for 20.4 hours with approximately 0.95 cc. of air per gram of oil per minute. The viscosity of the oil after oxidation was 648 SUS at 210° F. The oxidized oil containing barium was extracted with liquid propane at 123° F. and 250 p.s.i.g., using a propane to oil ratio of 6:1. The propane insoluble portion represented 36 percent by weight of the oil.

#### Example II

##### EVALUATION OF ADDITIVES

The modified diesel L-1 test referred to in this and other examples was carried out for a period of 60 or 120 hours, as indicated, instead of the 480 hours prescribed by the full scale diesel L-1 test set forth in "C.R.C.

Handbook 1946" by the Coordinating Research Council, Inc., at pages 347 and following, and as given in application Serial No. 304,659, page 25. In the 60-hour tests, a 1.0 percent sulfur fuel was used instead of the 0.4 percent used in the 120 hour test.

A 5 percent blend was made of barium detergent (prepared as described in Example I) in the base oil described in the above paragraphs. 1.25 percent of Lubrizol 309, a commercial antioxidant containing zinc dithiophosphate, was also added to the base oil. The following results were obtained in the diesel tests:

| 60 Hour Diesel Test |      | 120 Hour Diesel Test |
|---------------------|------|----------------------|
| Overall Rating..... | 95.2 | 90.1                 |
| Lacquer Rating..... | 91.1 | 83.7                 |
| Carbon Rating.....  | 99.0 | 95.0                 |

#### Example III

##### PREPARATION OF ADDITIVES

To a 50-gallon horizontal still was charged 340 pounds of a Mid-Continent oil, solvent refined and dewaxed, having a viscosity of 208 SUS at 210° F. This direct fired, batch still was equipped with a 1/4" stainless steel tubing containing 1/16" holes at 3 inch intervals for air distribution. The oil was heated to 482° F. at atmospheric pressure and then oxidized by passing air through the mass at 14 standard cubic feet per minute for a total of 7 hours. The viscosity of the resulting oxidized oil was 650 SUS at 210° F.

The resulting oxidized oil (305 pounds) was transferred to an open top, steam jacketed tank, heated to 170° F. and 9.25 pounds of finely ground (in a hammer mill) barium hydroxide octohydrate was added while the oxidized oil was being agitated. Two hours were allowed for the reaction. The barium treated oxidized oil was filtered using a horizontal plate Sparkler Filter maintained at about 325° F. The total filtrate weighed 293 pounds. The viscosity of the filtrate was 2740 SUS at 210° F. The barium treated oxidized oil was extracted by the batch method with 10 volumes of isobutane for 1 volume of the treated oil at 123° F. A yield of 30 percent insoluble material was obtained. This material was difficultly soluble in oil and had a sulfated ash equivalent to 6.8 percent barium hydroxide.

#### Example IV

##### EVALUATION OF ADDITIVE

A 5 percent blend was made of the isobutane-insoluble fraction of the barium treated oxidized oil (prepared as described in Example III) in the base oil described in Example II. 1.25 percent of Lubrizol 309, a commercial anti-oxidant containing zinc dithiophosphate, was also added to the base oil. The following results were obtained in the 60 hour diesel test:

|                     |      |
|---------------------|------|
| Overall rating..... | 86.8 |
| Lacquer rating..... | 78.9 |
| Carbon rating.....  | 93   |

#### Example V

820 grams of an ashless detergent, prepared by air oxidation at 482° F. and 25 p.s.i.g., followed by propane fractionation, as described in application Serial No. 304,659, was placed in a container and dissolved in 1400 ml. of benzene and 120 ml. of isopropyl alcohol. Thirty-eight grams of barium hydroxide octohydrate was added, which is 2.5 weight percent of the additive calculated as Ba(OH)<sub>2</sub>. The mixture was warmed just below boiling for one hour and then heated to azeotrope off the water and alcohol. Fresh portions of benzene were added to keep the material in solution. After the complete removal of the water, the solution was centrifuged to remove insolubles. A weighed amount of oil was added to

75 the solution and the benzene flashed off. This product

the solution and the benzene flashed off. This product gave the following results in the L-1 60 hour high sulfur fuel test using 1.25 percent Lubrizol 309 inhibitor, a commercial antioxidant containing zinc dithiophosphate. For comparison, the value for the untreated ashless detergent is also presented.

| Percent Concentration | Treated with Ba(OH) <sub>2</sub> | Piston Rating |         |        |
|-----------------------|----------------------------------|---------------|---------|--------|
|                       |                                  | Overall       | Lacquer | Carbon |
| 5.0.....              | No.....                          | 89.3          | 88.3    | 93.0   |
| 2.5.....              | Yes.....                         | 89.0          | 88.9    | 91.4   |
| 5.0.....              | Yes.....                         | 92.0          | 91.2    | 89.0   |

15 These results indicate that a 2.5 percent concentration of the barium hydroxide treated detergent is as effective as a 5.0 percent blend of the ashless detergent. A 5 percent blend of the treated detergent showed a very substantially improved lacquer rating. The ash content of the additive is about 2.8 percent, which amounts to only 0.14 percent ash in a 5 percent blend.

#### Example VI

25 A quantity of ashless detergent was prepared according to the method of application Serial No. 304,659 by oxidizing a finished 250 stock having a viscosity of 205 SUS at 210° F., using a temperature of 485° F. to 500° F., and a pressure of approximately 25 p.s.i.g. for 7 to 14 hours with air as the oxidant.

30 This ashless detergent was dissolved in a mixture of benzene and a small amount of isopropyl alcohol, and a calculated amount of the barium hydroxide dissolved in water was added to the solution. The mixture was heated at 140° to 160° F. for an hour. The water and alcohol were then removed as an azeotrope and the benzene solution centrifuged to remove the insoluble material. The solution was then mixed with oil and the benzene evaporated.

35 The results of modified EX-2 tests, described below, with these additives, are found in the following table. All tests were made using 1.25 percent Lubrizol 309, a commercial antioxidant containing zinc dithiophosphate and SAE 30 oil with 10 percent concentration of the additive, with the exception that the additive treated with 45 2.5 percent Ba(OH)<sub>2</sub> was used in a 11 percent concentration.

| Additive                                    | Oil Ring Plugging | Piston Varnish | Oil Screen | Total Varnish | Total Sludge |
|---------------------------------------------|-------------------|----------------|------------|---------------|--------------|
| Ashless Detergent                           | 9.0               | 7.8            | 8.0        | 40.3          | 14.7         |
| Treated with 0.5% Ba(OH) <sub>2</sub> ..... | 9.5               | 7.9            | 8.5        | 40.4          | 28.1         |
| Treated with 2.5% Ba(OH) <sub>2</sub> ..... | 9.5               | 8.5            | 9.0        | 43.5          | 32.8         |

50 The one digit ratings are from 0 to 10 and the two digit ratings are 0 to 50, the higher numbers being perfect. The fuel used was a thermally cracked "dirty-type" test fuel.

60 The EX-2 test is designed to give accelerated low temperature sludge conditions of a type found in city delivery service. The piston rings of the Chevrolet engine were slotted to allow a large amount of blow-by products to enter the oil and a dirty fuel is used. The test is of 96 hours' duration and, at the end of this period, the engine is rated for cleanliness and the oil for viscosity increase, sludge formation, etc. Under these conditions, the ashless detergent without further treatment consistently 70 caused an excessive thickening of the crankcase oil.

65 The product obtained by treating the ashless detergent with 2.5 percent Ba(OH)<sub>2</sub> showed a great improvement over the ashless detergent. Unlike the other samples tested, this additive, in a paraffinic oil and with a "dirty fuel," produced no crackcase "gel."

## 15

## Example VII

800 grams of the ashless detergent prepared as described in Example VI was dissolved in 1200 ml. of benzene and 100 ml. of isopropyl alcohol. To this mixture was added amounts of various bases equivalent to 2.5 weight percent of barium hydroxide in about 70 ml. of water. The mixture was heated below the boiling point for 1.5 hours and then the alcohol and water were removed as an azeotrope. The solution was centrifuged to remove the insolubles. The solution was diluted with SAE 20 oil. The benzene was evaporated, leaving the product.

The results of the L-1 60 hour high sulfur fuel engine tests are presented in the following table. All of the materials were tested at 5 percent concentration with 1.25 percent Lubrizol 309.

| Additive                                         | Piston Rating     |                   |        |
|--------------------------------------------------|-------------------|-------------------|--------|
|                                                  | Overall           | Lacquer           | Carbon |
| Ashless Detergent                                | <sup>1</sup> 87.2 | <sup>1</sup> 82.6 | 95.2   |
| Detergent Treated with 2.5% Ba(OH) <sub>2</sub>  | 92.0              | 91.2              | 89     |
| Detergent Treated with 1.6% KOH <sub>2</sub>     | 85.7              | 80.1              | 87     |
| Detergent Treated with 0.7% LiOH <sup>2</sup>    | 78.3              | 68.6              | 82     |
| Detergent treated with 1.08% Ca(OH) <sub>2</sub> | 91.3              | 83.9              | 98     |

<sup>1</sup> Average of four tests.

<sup>2</sup> Equal to 2.5 percent Ba(OH)<sub>2</sub> on a gram-equivalent basis.

The data in this example show that treating with alkali metal hydroxides does not result in the improvement shown when using alkaline earth metal hydroxides.

## Example VIII

Solvent refined 250 lubricating oil was agitated with an equal volume of 32 to 34 percent nitric acid at a temperature of 140 to 160° F. for 4 to 12 hours. The oil was separated, washed with cold water, and then dissolved in pentane. The emulsion was broken by the addition of isopropyl alcohol. Pentane was evaporated and a dark red oil recovered. 150 grams of this material was heated to 212° F., 3.75 grams of Ba(OH)<sub>2</sub>·H<sub>2</sub>O were added and the mixture heated for one hour at this temperature. Thereafter, the temperature was raised to 300° F. for an additional hour. The material, when cooled, was dissolved in pentane, centrifuged, and the solvent evaporated. The results of a Lauson engine test made with 1.75 percent concentration of the additive and 0.82 percent Santolube 395-X inhibitor, a commercial inhibitor containing P<sub>2</sub>S<sub>5</sub> reacted terpene with a control comprising the base oil appears in the following table.

Material tested:

|                              |     |
|------------------------------|-----|
| Base oil                     | 6.3 |
| Base oil with above additive | 8.0 |

In the above examples, the mixtures were agitated in order to keep the alkaline earth compounds in suspension, since these materials, which are powders, tend to settle out of the solution instead of remaining uniformly dispersed and in good contact with the oil. In the drawing which accompanies and forms a part of this disclosure, I have illustrated apparatus for preparing the detergents of this invention, this apparatus taking advantage of the fact that an oxidized oil percolating over an alkaline earth metal hydroxide reacts with the material to form the additive.

This apparatus comprises an elongated vessel 10 provided with an oil inlet 11 and a gaseous material outlet 12 in the upper end portion thereof. Vessel 10 is filled with an inert granular support 13, such as bauxite, on which has been deposited the desired basic material, such as an alkaline earth metal hydroxide, oxide, or carbonate. Heat exchangers 14, 16 and 17 are positioned within this bed in order to maintain the temperature desired for treatment. Means for introducing gaseous material is provided in a lower portion of vessel 10, this being intro-

## 16

duced through line 18 to a perforated plate 19, or other equivalent gas distribution means.

Conduit 21 communicates with the lower portion of vessel 10 and extends to the central or upper portion of liquid-liquid extraction zone 22. From the lower end portion of zone 22, conduit 23 extends to fractionator 24, this fractionator being provided with conduit 26 extending from the lower portion thereof. Extending from the upper end portion of zone 22 there is provided conduit 27 which 10 communicates with fractionator 28, this fractionator 28 being provided with conduit 29 extending from the lower end portion thereof. Conduit 31 extends from the upper portion of fractionator 24 to the lower end portion of extraction zone 22 and conduit 32 extends from the upper portion of fractionator 28 to conduit 31. Make-up solvent can be added through conduit 33.

In the operation of this apparatus, the oil to be oxidized is introduced through conduit 11 into the upper portion of vessel 10, this vessel being filled with the treating material:

20 The oil passes downwardly over this granular treating material 13 countercurrent to the flow of oxidant introduced through distribution means 19. The oil is added at such a rate that it is oxidized to the desired extent by the time it leaves vessel 10, it being removed through conduit 21. 25 The use of this apparatus provides continuous movement downwardly over the treating material with a minimum of mixing of the various portions of the oil, a situation that is difficult to avoid when batch-wise operation is utilized. Since the specific gravity of the oxidized material is higher than that of the charge oil, the tendency of these materials to mix is minimized. For instance, with one particular oil, the oxidized material had a specific gravity of 0.93 compared to 0.87 for the charge oil.

30 The apparatus shown in this drawing includes the propane fractionation step which is preferred in the recovery of the additive. The treated oil is introduced by conduit 21 into liquid-liquid extraction zone 22 and conduit 31 supplies solvent thereto. Although the treated oil and solvent can be introduced at a common point I prefer to operate by introducing the oil into the central or upper portion of zone 22 and by supplying the solvent to the lower portion, as shown, in order to provide countercurrent extraction. Temperatures for the oxidation have been previously recited. Temperatures in the extraction zone can vary widely. It is preferred to operate below the critical temperature with liquid phase conditions. Using propane as the solvent, a suitable range for the bottom of the zone is 100 to 150° F., preferably 45 about 110° F., and the range of 125 to 200° F., preferably about 150° F., for the top of the zone. The non-soluble portion of the treated stock, being heavier, is removed from the lower portion of zone 22, conveyed by line 23 to fractionator 24, where the solvent dissolved 50 therein is returned to the process through overhead conduit 31 and the additive is recovered as a bottom product in conduit 26. The propane soluble portion, the upper layer found in the zone 22, is passed to fractionator 28 through conduit 27, where the propane is recovered 55 and returned to the system through line 32 and the un-oxidized portion is recovered in conduit 29. This portion can be returned to the treating column 10, as desired, or used for other purposes.

As many possible embodiments may be made of this 60 invention without departing from the spirit and scope thereof, it is to be understood that all matter herein set forth or shown in the accompanying drawing is to be interpreted as illustrative and not in a limiting sense.

I claim:

70 1. A process for producing a material having detergent and dispersant properties which comprises subjecting a hydrocarbon fraction, having a refractive index  $n_D^{20}$  of between 1.440 and 1.520, a minimum molecular weight of 450, a viscosity of at least 50 SUS at 210° F., a viscosity 75 index (when determinable) at at least 50, and an average

carbon atom content per molecule of at least 40, to oxidation with air at a temperature of 100° F. to 800° F. for a time of 3 to 75 hours and at a pressure of 10 to 200 p.s.i.a., said air being supplied at a rate of 0.01 to 3.0 cf. per hour per pound of said hydrocarbon, recovering the oxidized fraction of said hydrocarbon by solvent extraction, adding to said oxidized portion 0.1 to 20 percent by weight of at least one compound selected from the group consisting of alkaline earth hydroxides, oxides, and carbonates, heating said mixture at a temperature in the range of 50 to 500° F. for a time of 5 minutes to 5 hours, and recovering the resulting treated material, said material having detergent and dispersant properties in lubricating oil compositions.

2. The process of claim 1 in which said alkaline earth material is barium hydroxide.

3. The process of claim 1 in which said alkaline earth material is calcium hydroxide.

4. The process of claim 1 in which said alkaline earth material is barium oxide.

5. The process of claim 1 in which said alkaline earth material is calcium oxide.

6. A process for producing a material having detergent and dispersant properties which comprises subjecting a hydrocarbon fraction, having a refractive index  $n_D^{20}$  of between 1.440 and 1.520, a minimum molecular weight of 450, a viscosity of at least 50 SUS at 210° F., a viscosity index (when determinable) of at least 50, and an average carbon atom content per molecule of at least 40, to oxidation in the presence of an oxidizing agent under oxidizing conditions and at least one compound selected from the group consisting of alkaline earth hydroxides, oxides, and carbonates, said oxidation being sufficient to provide at least a 1.5 fold increase in viscosity, and recovering a resulting material having detergent and dispersant properties when used in a lubricating oil.

7. A lubricant composition comprising a major portion of lubricating oil and at least 0.1 percent by weight of an oil soluble material having detergent and dispersant properties, said material produced by oxidation and treatment with at least one compound selected from the group consisting of alkaline earth hydroxides, oxides and carbonates, of a hydrocarbon fraction having a refractive index  $n_D^{20}$  of between 1.440 and 1.520, an average molecular weight of at least 550 and no appreciable portion thereof having a molecular weight below 450, a viscosity of at least 50 SUS at 210° F., a viscosity index (when

determinable) of at least 50, and an average carbon atom content per molecule of at least 40, the solid oxidation product having an acid number below 50, a saponification number in the range of 0 to 100, and an oxygen content in the range of 1 to 15 percent by weight.

8. The composition of claim 7 in which said material having detergent and dispersant properties is present in an amount from 0.3 to 10.0 parts by weight.

9. A lubricant composition comprising a major portion of lubricating oil and at least 0.1 percent by weight of an oil-soluble material having detergent and dispersant properties, said material produced by oxidation and treatment with at least one compound selected from the group consisting of alkaline earth hydroxides, oxides, and carbonates, of a hydrocarbon fraction having a refractive index  $n_D^{20}$  of between 1.480 and 1.515, an average molecular weight of at least 600 and no appreciable proportion thereof having a molecular weight below 400, a viscosity of at least 100 SUS at 210° F., a viscosity index (when determinable) of at least 80, and an average carbon content per molecule of at least 50, the solid oxidation product having an acid number below 50, a saponification number in the range of 0 to 100, and an oxygen content in the range of 1 to 15 percent by weight.

10. The composition of claim 9 wherein said alkaline earth material is barium hydroxide.

#### References Cited in the file of this patent

#### UNITED STATES PATENTS

|    |           |                  |                |
|----|-----------|------------------|----------------|
| 30 | 2,015,347 | Luther et al.    | Sept. 24, 1935 |
|    | 2,070,567 | Adams            | Feb. 16, 1937  |
|    | 2,070,627 | Shoemaker        | Feb. 16, 1937  |
|    | 2,128,574 | Van Peski et al. | Aug. 30, 1938  |
| 35 | 2,252,087 | McNab            | Aug. 12, 1941  |
|    | 2,389,090 | Shields          | Nov. 13, 1945  |
|    | 2,653,909 | Frazier          | Sept. 29, 1953 |
|    | 2,682,553 | Kirk             | June 29, 1954  |
| 40 | 2,705,241 | McKinley et al.  | Mar. 29, 1955  |
|    | 2,726,255 | Walker et al.    | Dec. 6, 1955   |
|    | 2,955,084 | Bartleson et al. | Oct. 4, 1960   |

#### OTHER REFERENCES

45 "Petroleum Refiner," vol. 28, No. 9, September 1949, pages 87, 91 and 92.

"Performance of Lubricating Oils," Zuidema, Reinhold Pub. Co., 1952, page 123.